

## UNITED STATES PATENT OFFICE

2,309,102

## COPPER BASE ALLOY

Donald K. Crampton, Marion, and Henry L. Burghoff, Waterbury, Conn., assignors to Chase Brass & Copper Co. Incorporated, Waterbury, Conn., a corporation

No Drawing. Application August 16, 1941,  
Serial No. 407,218

4 Claims. (Cl. 148—32)

This invention relates to improvements in copper-base alloys.

One object of this invention is to provide improved copper-base alloys having good physical and corrosion-resistant properties.

Other objects of this invention will appear from the present disclosure.

We have invented improved copper-base alloys having tin from 2% to 10%, phosphorus from 0.05% to 0.3%, nickel from 0.35% to 2% with the phosphorus being from  $\frac{1}{3}$  to  $\frac{1}{10}$  of the nickel by weight, and the remainder substantially of copper, the copper being from 88% to 97.5%, and the total of the copper and tin being at least 97.5%. Another alloy range is to have the tin from 2% to 8%, the phosphorus from 0.05% to 0.3%, the nickel from 0.35% to 1.5%, and the balance substantially of copper, the copper being from 90% to 97.5%, and the total of the copper and tin being at least 97.5%. One preferred alloy is tin about 2%, phosphorus about 0.2%, nickel about 1%, and the balance substantially of copper. Another preferred alloy is tin about 5%, phosphorus about 0.1%, nickel about 0.5%, and the balance substantially of copper.

If any lead is to be present in the alloy, it should not exceed 1.5% as it embrittles the alloy so as to interfere with metal working operations used in producing wrought articles and shapes from the alloy. If any aluminum or silicon or chromium is to be present in the alloy, the amount of the aluminum or silicon or chromium should not exceed 0.1% as these elements result in refractory and abrasive oxides which cause rapid wear on the fabricating tools and dies.

These alloys are age-hardenable and possess desirable high yield-strength with good ductility and tensile strength in their age-hardened condition. They also have excellent wear-resistance and excellent spring-making properties with less cold-working than is necessary with ordinary tin bronzes of similar tin content. They also have good corrosion-resistance to saline solutions.

The alloys of the invention can be rendered soft and ductile by annealing or heating at temperature in the range from about 1200° F. to about 1600° F. to constitute a solution treatment for the age-hardening nickel and phosphorus material, and quenching or cooling sufficiently rapidly from such temperature to hold age-hardening material in solution, and can be subsequently age-hardened by re-heating or aging at temperature in the range from about 600° F. to about 1050° F. for from about one-half to six hours or longer, depending on the temperature,

to precipitate age-hardening material out of solution.

One notable thing about the alloys of this invention is that those of lower tin content achieve as high hardness and strength as those of higher tin content, when in the age-hardened condition. This is remarkable for it is well known that the hardness and strength of ordinary tin bronze increases with tin content. This important fact concerning our improved alloys makes possible a considerable saving in alloy cost due to the saving of costly tin, and in production cost, for the alloys of higher tin content are ordinarily processed only with difficulty.

15 The invention may be carried out in other specific ways than those herein set forth without departing from the spirit and essential characteristics of the invention, and the present embodiments are, therefore, to be considered in all respects as illustrative and not restrictive and all changes coming within the meaning and equivalency range of the appended claims are intended to be embraced therein.

We claim:

25 1. A hardened copper-base alloy consisting substantially of: tin from 2% to 10%; phosphorus from 0.05% to 0.3%; nickel from 0.35% to 2% with the phosphorus being from  $\frac{1}{3}$  to  $\frac{1}{10}$  of the nickel by weight; and the balance substantially of copper, the copper being at least 88% and the total of the copper and tin being at least 97.5%; and the alloy having been given a solution treatment by having been suitably cooled from temperature in the range from about 1200° F. to about 1600° F. and having been hardened by having been given a precipitation treatment at temperature in the range from about 600° F. to about 1050° F.

2. A hardened copper-base alloy consisting substantially of: tin from 2% to 8%; phosphorus from 0.05% to 0.3%; nickel from 0.35% to 1.5% with the phosphorus being from  $\frac{1}{3}$  to  $\frac{1}{10}$  of the nickel by weight; and the balance substantially of copper, the copper being at least 90% and the total of the copper and tin being at least 97.5%; and the alloy having been given a solution treatment by having been suitably cooled from temperature in the range from about 1200° F. to about 1600° F. and having been hardened by having been given a precipitation treatment at temperature in the range from about 600° F. to about 1050° F.

40 3. A hardened copper-base alloy consisting substantially of: tin about 2%; phosphorus about 0.2%; nickel about 1%; and the balance sub-

stantially of copper, the total of the copper and tin being at least 97.5%; and the alloy having been given a solution treatment by having been suitably cooled from temperature in the range from about 1200° F. to 1600° F. and having been hardened by having been given a precipitation treatment at temperature in the range from about 600° F. to about 1050° F.

4. A hardened copper-base alloy consisting substantially of: tin about 5%; phosphorus about 0.1%; nickel about 0.5%; and the balance sub-

5

10

stantially of copper, the total of the copper and tin being at least 97.5%; and the alloy having been given a solution treatment by having been suitably cooled from temperature in the range from about 1200° F. to about 1600° F. and having been hardened by having been given a precipitation treatment at temperature in the range from about 600° F. to about 1050° F.

DONALD K. CRAMPTON.  
HENRY L. BURGHOFF.